

May 10, 1949.

F. G. BROCKMAN ET AL

**2,469,947**

## PRODUCTION OF EXTREMELY THIN FILAMENTS

Filed April 13, 1944

FIG. 1



FIG. 2



INVENTOR.  
FRANK G. BROCKMAN  
JOHN W. WESCOTT, 2<sup>ND</sup>

BY JOHN W. WEScott, 2<sup>nd</sup>

BY *JOHN W. HENRY,*

James G. Cleveland.

**ATTORNEY**

## UNITED STATES PATENT OFFICE

2,469,947

## PRODUCTION OF EXTREMELY THIN FILAMENTS

Frank G. Brockman, Woodbury, and John W. Wescott, 2nd, Chatsworth, N. J., assignors to Socony-Vacuum Oil Company, Incorporated, a corporation of New York

Application April 13, 1944, Serial No. 530,950

1 Claim. (Cl. 204—12)

**1**  
This invention relates generally to a method of producing ribbon-like filaments and more particularly to a method of producing extremely fine filaments. A specific application for such filaments can be of use in bolometers, thermocouples, or other measuring instruments employed where it is desired to detect and/or measure extremely small amounts of radiant energy.

In the prior art workers have prepared similar filaments by using Wollaston wire and removing the silver from the thin platinum core by the action of nitric acid; or by welding platinum foil to heavier silver foil and rolling this double foil to suitable thickness, cutting out ribbons and then dissolving away the silver with nitric acid; or by electroplating nickel upon stainless steel, mechanically removing the thin nickel plate and cutting the resultant thin foil into filaments. The first two methods present numerous difficulties, not the least of which is the effect of gas evolution upon the filament during the acid treatment. The last method is obviously very difficult when the foil is extremely thin.

The method of the instant invention is free of the difficulties inherent in those of the prior art enumerated above; is based on sound electrochemical principles; and produces extremely thin filaments with considerably greater ease than any of the previous methods.

Broadly stated the method of the present invention comprises plating the metal selected for the filaments on a sheet of base metal, cutting the composite metal sheet into ribbons, securing each ribbon to a frame to form a voltaic couple, and immersing the frames and ribbons carried respectively by each frame into an aqueous bath of a cyanide of an alkali metal whereby the base metal is electrolytically dissolved.

Therefore, the primary object of the present invention resides in the provision of a method of producing extremely thin filaments having uniform physical, thermal and electrical characteristics.

Another object of this invention resides in the production of filaments having a thickness of approximately 0.1 micron (approx.  $\frac{1}{1000000}$  inch) which is uniform throughout.

Still another object of this invention resides in the provision of a method of electrolytically producing extremely thin metal filaments without the evolution of gases in the vicinity of the filament.

This invention further contemplates the use of a voltaic couple in electrolytically dissolving the base metal from the filament metal.

**2**  
Still another object of the present invention resides in the provision of a method of production of extremely thin filaments whose thickness can be duplicated with accuracy.

5 This invention further contemplates a method of producing extremely thin filaments that can be practiced economically and with facility.

Other objects and advantages of the present invention will become apparent from the following detailed description when considered with the drawings, in which

Figure 1 is a longitudinal view of the frame and ribbons shown in part in vertical section; and

15 Figure 2 is another longitudinal view of the frame and ribbons differing from that of Figure 1 in that the vertical section is taken at right angles to that shown in Figure 1.

16 Figure 3 is a view of the frame and ribbons in the bath.

20 According to electrochemistry, if a voltaic couple formed by two metals that differ widely in the electrochemical series, is immersed in an aqueous solution of a cyanide of an alkali metal, the metal of the couple having the more positive position in the electrochemical series will be dissolved. The chemical reaction that takes place is that the +ions of the metal having the more positive position in the electrochemical series will enter the aqueous solution and will react with the negative cyanide ions to form a complex with the cyanide. The positive ions of the alkali metal used migrate to the metal of the couple having the most negative chemical potential where they pick up negative charges and react with water forming stable hydrogen. The stable hydrogen is evolved from that electrode in the form of gas. This reaction will continue until the metal of the couple having the most positive position in the electrochemical series has been completely dissolved.

25 Reaction at the copper electrode:



30 Reaction at the platinum electrode:



35 It will be understood that the metals selected for the voltaic couple should be separated by a fairly large potential difference in the voltaic

order of metals in aqueous solutions of a cyanide of an alkali metal.

Utilizing the above theory, a base metal, such as copper, is selected. This metal should be in the form of, or reduced to, a sheet of foil having a moderate thickness, for example, 0.0015 inch. Then the metal from which the thin filaments are to be formed is selected, for example, nickel. The procedure then consists in plating the copper foil with the nickel to a thickness equal to that desired in the final filament by using any of the well-known electroplating methods. Although it is possible to deposit the nickel on the copper foil by other methods such as evaporation or sputtering, the plating process is the preferable one because of the ease with which a coating of the desired thickness can be applied.

After the nickel is deposited on the copper to the desired thickness ribbons of the required width and length are cut. These ribbons are mounted in a frame or frames, as shown in Figures 1 and 2, by any appropriate means, such as soldering. This frame serves as a support for the final filament or filaments.

Referring to the drawings, particularly Figures 1 and 2, the copper-nickel ribbon 10 is mounted in the platinum frame by soldering the nickel side of the ribbon at each end to the ends of platinum wires 11 and 12. Wires 11 and 12 are held in spaced relationship by glass beads 13 and 14. A third platinum wire 15 is also held in parallel spaced relationship by the glass beads 13 and 14. This wire is electrically connected to the center of the nickel side of the ribbon 10 by soldering the nickel to the platinum bridge 16. The free ends of all three wires 11, 12 and 15 extend through openings in the glass plug 17. Each wire is sealed in its opening.

As shown in Figure 3 the assembled ribbon and platinum frame is submerged in a bath 18 formed of a cyanide of an alkali metal.

Obviously the platinum frame can be formed in other configurations. The one disclosed is that used in the manufacture of bolometer ribbons and which was carried over into a finished instrument where it served as a permanent support for the ribbons and means for making electrical circuit connections to them.

The copper foil is now dissolved, leaving the thin layer of nickel which was originally deposited on the copper foil. This is accomplished by immersing the ribbon while mounted in its frame in an aqueous solution of a cyanide of an alkali metal such as potassium or sodium, and making a metallic connection between the ribbon, by way of the frame, and an electrode of platinum, which is immersed in the same solution, to form a voltaic couple. The concentration of the aqueous solution of a cyanide of an alkali metal is not critical but affects the time required to complete the process. It is obvious that a mere trace of a cyanide of an alkali metal would unduly prolong the process. If the frame is constructed of platinum, the electrode is superfluous. The couple formed by the platinum and the copper acts electrolytically, the copper being dissolved away without the evolution of gas, which is so destructive to the thin nickel filament. Copious gassing occurs at the platinum, but this is not objectionable since the gas does not come into contact with the thin filament of nickel. When all of the copper is dissolved, gassing at the platinum electrode ceases, and the extremely thin filament of nickel in its mounting frame is obtained.

In practicing the above-described method, a number of extremely thin filaments have been prepared. A typical example of these is a pair of nickel filaments that were simultaneously produced each of which had the following properties:

Length, 1.4 cm.

Width, 0.038 cm.

Thickness, 0.1 micron (approx.  $4/1000000$  inch).

Although filaments having comparable dimensions to those of the example cited above are being used in bolometer detectors for infra-red spectrometers, it is obvious to those skilled in the art that they can be used anywhere that it is desired to measure extremely small amounts of radiant energy.

This method is also applicable to the production of extremely sensitive thermocouples that are adapted for use in measuring radiant energy. A foil of base metal is first plated with one of the metals of which the finished thermocouple is formed. The plating should cover a little over one-half of the foil. Next, the second metal of which the finished thermocouple is formed is plated over the other end of the base metal foil. This plating should slightly overlap the first plating. Now, if the two metals, plated on the base metal, are more negative than the base metal, it is possible to etch away the base metal in the manner described above in connection with the extremely fine ribbon-like filaments.

We claim:

In a method of producing an extremely thin nickel filament by plating nickel on copper foil to a thickness of 0.1 micron, cutting the plated foil to form a ribbon having the length and width of the desired finished filament, and dissolving the copper foil from the nickel filament by submerging the composite ribbon in a bath formed of an aqueous solution of a cyanide of an alkali metal, the improvement which comprises securing the ribbon to a platinum frame in conducting relationship therewith before it is submerged in the bath to form a voltaic couple, whereby on submerging the frame and ribbon in a bath the copper will be dissolved and bubbling occasioned by liberation of hydrogen during dissolution of the copper will occur only at the platinum electrode of the voltaic couple.

FRANK G. BROCKMAN.  
JOHN W. WESCOTT, 2ND.

#### REFERENCES CITED

The following references are of record in the file of this patent:

#### UNITED STATES PATENTS

| Number    | Name              | Date           |
|-----------|-------------------|----------------|
| 771,340   | Van Housen et al. | Oct. 4, 1904   |
| 865,688   | Edison            | Sept. 10, 1907 |
| 909,831   | Stricker-Auermann | Jan. 13, 1909  |
| 1,709,801 | Muller            | Apr. 16, 1929  |
| 1,787,139 | Cain              | Dec. 30, 1930  |
| 2,052,962 | Booe              | Sept. 1, 1936  |

#### OTHER REFERENCES

A Comprehensive Treatise on Theoretical and Inorganic Chemistry by J. W. Mellor, vol. III, Longmans, Green & Co., New York, 1923, pages 502, 503.

**Certificate of Correction**

May 10, 1949.

Patent No. 2,469,947.

FRANK G. BROCKMAN ET AL.

It is hereby certified that errors appear in the printed specification of the above numbered patent requiring correction as follows:

Column 2, line 52, strike out that portion of the formula reading



and insert the same above “Reaction at the platinum electrode:” in line 46; and that the said Letters Patent should be read with these corrections therein that the same may conform to the record of the case in the Patent Office.

Signed and sealed this 18th day of October, A. D. 1949.

[SEAL]

THOMAS F. MURPHY,  
*Assistant Commissioner of Patents.*